

Oct. 24, 1933.

J. H. DE BOER ET AL

1,931,647

PROCESS FOR INTRODUCING ACTIVE METAL INTO A VACUUM TUBE

Filed Nov. 13, 1931



INVENTOR  
J.H. DE BOER J.L.H. JONKER  
BY & K.M. VAN GESSEL

*J.H. De Boer*  
ATTORNEY

## UNITED STATES PATENT OFFICE

1,931,647

## PROCESS FOR INTRODUCING ACTIVE METAL INTO A VACUUM TUBE

Jan Hendrik de Boer, Johan Lodewijk Hendrik Jonker, and Karel Marinus van Gessel, Eindhoven, Netherlands, assignors to Radio Corporation of America, a corporation of Delaware

Application November 13, 1931, Serial No. 574,810,  
and in the Netherlands November 15, 1930

7 Claims. (Cl. 250—27.5)

This invention relates to a process for introducing a chemically active metal into an electron discharge tube. Among such metals the alkaline earth metals and the alkali metals play a prominent part, and are frequently used for producing an electron emitting layer on a cathode, and also for binding residual gases or gaseous impurities.

Owing to the great affinity of these metals for oxygen they cannot be exposed to the open air. For this reason various methods have already been proposed for introducing these metals into a vacuum tube without running the risk of the metals being attacked by the oxygen of the air. It has already been proposed to introduce the active metal into the discharge tube by introducing compounds of the metal from which the metal may be liberated by heating and which themselves are not attacked by the air, the compounds being heated and decomposed after evacuation of the tube. For introducing alkaline earth metals use has been made, for example, of compounds such as azides of these metals.

Instead of decomposable compounds use has been made of alloys for example, magnesium and aluminum alloys of the active alkaline earth and alkali metals. In these alloys the accompanying metal protects against oxidation the active metal to be introduced into the tube whilst the accompanying metal either volatilizes when the alloy is heated and decomposed in the discharge tube, or stays behind at the point at which the decomposition takes place.

Furthermore it has been proposed to introduce compounds of active metals together with a suitable reducing agent into a discharge tube and to reduce these compounds after exhaustion of the tube. It has been proposed, for example, to bring a mixture of caesium chloride or barium oxide and magnesium, calcium or zirconium into a discharge tube and to heat this mixture after exhaustion of the tube to such a temperature that the caesium or barium is produced in the form of vapour.

When using these methods the substances to be introduced into the discharge tube are often shaped as pellets and fixed in this form to one of the metal members of the discharge tube.

Though excellent results have been obtained with some of the methods above referred to, it has been found that they do not always give perfectly satisfactory results. If, for example, the cathode of a triode is coated with a layer of barium introduced in the triode by means of

such a pellet, then the use of this triode is often attended with disturbances in the discharge manifested for example, by cracking noises in a loudspeaker connected to the triode.

According to the invention these difficulties are avoided by introducing into the tube the active metal, or a compound or alloy from which this metal may be produced, admixed with such a quantity of insulating material that the introduced mixture is electrically insulating even after it is heated to produce the active metal. In fact, it has been found that the said disturbances are due to coherent particles of the compound introduced into the tube and from which the active metal is produced. On heating the compound and volatilizing the produced metal particles of the introduced mass or compound seem to scale off. These particles may lodge, for example, between the electrodes of the tube and make an electrical connection between the electrodes.

By mixing the metal to be introduced into the tube, or the compound or alloy from which this metal may be produced with a sufficient quantity of an insulating material, it is found that even if particles do scale off from the introduced mass no conducting connections can be formed by said particles. The material to be introduced must be substantially an insulator, i. e. it must have such a high resistance that the voltages present in the vacuum tubes do not cause an appreciable current to flow thru the material.

The invention will be more clearly understood by reference to the accompanying drawing which represents by way of example an electron discharge tube embodying the invention.

The triode shown on the drawing has a vitreous envelope 1, in which an anode 2, a grid 3 and an electron emitting cathode 4 are enclosed. The anode has an aperture in front of which a receptacle 5 is fixed on the anode. If desired, the side of this receptacle facing the interior of the anode may be covered by a netting or mesh screen. The receptacle contains a mixture of the active metal and an insulating material, such as barium mixed with magnesium oxide or zirconium oxide preferably finely divided or powdered. The percentage of oxide is so chosen that the mixture which is preferably, and by the aid of a binder, if necessary, brought into a coherent form for example, that of a pellet, is electrically insulating. After the exhaustion of the tube the receptacle 5 is heated, which may be done by means of a high frequency magnetic field until the barium is expelled from the mix-

ture. Part of this expelled barium deposits on the cathode 4, where it forms a layer which after being oxidized, if desired, is electron emitting.

The mixture introduced into the receptacle 5 may be prepared by mixing barium azide with a sufficient quantity of magnesium oxide or zirconium oxide and by heating this mixture in a vacuum or in an inert atmosphere to such a temperature that the barium azide decomposes 10 leaving barium and liberating nitrogen. However, the temperature to which the mixture is heated is kept so low that all or at least a large part of the barium produced stays behind in the mixture. In this way there is obtained a mixture 15 of magnesium oxide or zirconium oxide intimately admixed with finely divided metallic barium. As has been stated the starting mixture is so proportioned that the prepared mixture is electrically insulating. Good results have 20 been obtained, for example, from a starting mixture of barium azide and magnesium oxide or zirconium oxide, in which the ratio by weight between the barium azide and the magnesium oxide or zirconium oxide is 1 to 15.

25 It is also possible to decompose the barium azide after the mixture has been introduced into the discharge tube. In this case the nitrogen is liberated in the discharge tube and must be removed by a vacuum pump.

30 This mixture to be introduced into the vacuum tube may be conserved in a vacuum or under a protecting liquid. It is possible to expose the mixture to the open air for a short time without the active metal contained in the mixture being 35 materially attacked by the oxygen of the air. The barium oxide produced in the mixture by exposure to the air does not unfavorably affect the conductivity of the mixture introduced into the tube, since barium oxide is practically an insulator under these conditions. In preparing 40 this mixture one may also start with barium oxide and a reducing agent, provided care be taken that a sufficient excess of barium oxide is present in which case the prepared mixture will 45 contain free barium, barium oxide and the oxide of the reducing agent.

We claim:

1. The method of introducing a chemically active metal into an evacuated electric discharge 50 device which consists in providing within said

device a mixture of the active metal and a refractory insulating material sufficient in amount to render said mixture electrically insulating, and heating said mixture to vaporize some of said metal.

2. An electric discharge device containing a mixture of a chemically active metal and a refractory insulating material sufficient in amount to render said mixture electrically insulating, and means whereby said mixture may be heated to vaporize some of said metal.

3. The method of introducing barium into an evacuated electron discharge device which consists in placing within said device in position to be heated a mixture of barium in finely divided form and a powdered zirconium oxide sufficient in amount to render said mixture electrically insulating, and heating said mixture to vaporize some of said barium.

4. The method of introducing barium into an evacuated electric discharge device which consists in placing within said device in position to be heated a mixture of barium in finely divided form and powdered magnesium oxide sufficient in amount to render said mixture electrically insulating, and heating said mixture to vaporize some of said barium.

5. The method of preparing a clean up agent which consists in mixing a refractory insulating material and a compound of a chemically active metal decomposable by heat into metal and reaction products, and heating said mixture to decompose said compound and to produce the active metal in finely divided form intimately mixed with and distributed thru said insulating material.

6. A clean up agent for electron discharge devices comprising a pellet of a mixture of an alkaline earth metal and an insulating oxide sufficient in amount to make said mixture substantially an electrical insulator.

7. A clean up agent consisting of an electrically insulating mixture of a finely divided barium compound and powdered magnesium oxide the ratio by weight being 1 of the former to 15 of the latter.

JAN HENDRIK DE BOER.  
JOHAN LODEWIJK HENDRIK JONKER.  
KAREL MARINUS VAN GESSEL.

125

55

136

60

138

65

140

70

145

75

150